

V. C. GOODRIDGE,  
REVERSIBLE BATTERY,  
APPLICATION FILED JULY 3, 1922.

1,436,873.

Patented Nov. 28, 1922.

3 SHEETS—SHEET 1.

FIG. 2



FIG. 1



INVENTOR:  
Victor C. Goodridge  
BY Jno. S. Elliott  
ATTY

1,436,873.

V. C. GOODRIDGE.  
REVERSIBLE BATTERY.  
APPLICATION FILED JULY 3, 1922.

Patented Nov. 28, 1922.

3 SHEETS—SHEET 2.



INVENTOR:  
Victor C. Goodridge  
By Jno. G. Elliott  
ATTY.

V. C. GOODRIDGE.  
REVERSIBLE BATTERY.  
APPLICATION FILED JULY 3, 1922.

1,436,873.

Patented Nov. 28, 1922.

3 SHEETS—SHEET 3.

Fig. 9.



Fig. 10



Fig. 11.



Inventor:

<sup>13</sup> Victor C. Godridge

By Irving Elliott Attty.

## UNITED STATES PATENT OFFICE.

VICTOR C. GOODRIDGE, OF CHICAGO, ILLINOIS, ASSIGNOR TO GOODRIDGE BATTERY CO.,  
A CORPORATION OF ILLINOIS.

## REVERSIBLE BATTERY.

Application filed July 3, 1922. Serial No. 572,589.

*To all whom it may concern:*

Be it known that I, VICTOR C. GOODRIDGE, a citizen of the United States, and a resident of Chicago, in the county of Cook and State of Illinois, have invented certain new and useful Improvements in Reversible Batteries, of which the following is a specification.

This invention relates to reversible batteries of the type disclosed in my pending application No. 531,120, filed January 23, 1922, and consists of certain improvements in said battery, all as hereinafter set forth, whereby the operation of the battery is improved and the durability of the cells is enhanced.

The nature of the improvements will be understood if reference is made to the accompanying drawings, constituting a part of this specification, in which,—

20 Figure 1 is a sectional view of the invention, taken on the line 1—1 of Figure 2;

Figure 2 is a sectional view taken on the line 2—2 of Figure 1;

25 Figure 3 is a sectional view of the receptacle used in connection with the invention;

Figure 4 is a top view of one form of the electrode employed in connection with the invention;

30 Figure 5 is a side elevation of such electrode;

Figure 6 is a top view of another form of the electrode used in connection with the invention;

35 Figure 7 is a side view of such electrode;

Figure 8 is a view, partly in section, of the vent tube employed in connection with the invention;

40 Figure 9 is a similar view of an electrolytic cell embodying further features of my invention in which ozone may be developed;

Figure 10 is a vertical sectional view of a primary cell embodying certain features of my invention; and

45 Figure 11 is a view of a volta pile embodying my invention.

The battery, as described in my pending application, consists of a receptacle 1 of hard rubber or glass, which is provided with an interior groove 2 for retaining a cover 14 of plastic material, and with spacing members 3 for the containers 4. These containers are made of cellulose, such as blotting paper, and, according to the present invention, are treated in a particular manner to increase

the effectiveness of the battery and to render 55 the containers inert as regards the action of the electrolyte.

Each of the containers 4 is filled, approximately, with a material 5, such as red lead,  $Pb_3O_4$ , for producing the positive electrode, 60 and the receptacle 1 is likewise approximately filled with a material 6, such as litharge  $PbO$ , for producing the negative electrode, these materials being, respectively, changed to  $PbO_2$  and  $Pb$ , when the battery 65 is charged by passing a current of electricity through it in the usual manner.

Disposed at opposite sides of the battery, are terminals 7 and 8, the terminal 7 having a plurality of legs or plates of lead, corresponding in number with their containers, the negative terminal 8 being similarly provided with legs or plates of lead, except as to the number employed, which is either one more or one less than the number of positive terminal legs. All of the terminal legs are surrounded by the electro-active materials, as will be understood. The electrolyte 6<sup>a</sup> may be sulphuric acid, or some equivalent substance.

70 The legs of each terminal are connected by a suitable bridge 9, and the terminals may be respectively provided with collars 10, 10 and slots 12, the collars 10 being embedded in plastic material 14, such as is used in capping batteries, and the slots 12 affording a convenient means for wiring the terminals. A support of hard rubber, or other inert material 13, resting on the bridges 9, underlies the terminals 7, 8, and sustains the 80 plastic material 14 until it hardens.

75 The battery is relieved of gases by a vent tube 15 having an aperture 16 and a perforated cap 17.

85 The improvements forming the subject matter of the present application relate to the general construction of the battery; to the treatment of the blotting paper or equivalent porous cellulose of which the containers 4 are composed; to the composition and 90 the treatment of the materials of the respective electrodes, and to the electrolyte.

95 Cellulose, in its natural condition, is carbonized by the spontaneous action of sulphuric acid and other electrolytes, a chemical reaction which reduces the efficiency of a battery. I have found that if cellulose containers are saturated with an aqueous solu-

tion of a metallic salt of the alkaline group, such as sodium silicate,  $\text{Na}_2\text{SiO}_3$ , this solution is electrolyzed these containers remain white instead of becoming black as they do when treated with sulphuric acid, and that the compositions formed outside and inside the containers are uncontaminated with resistant substances, such as sulphate of lead, produced in ordinary batteries by the action of the sulphuric acid, and that said battery is, consequently, capable of developing a current of unusually high amperage and voltage.

In constructing the battery, I produce a block of wood of the size of the containers, and fold around and under it, one at a time, pieces of white blotting paper, two or three layers being laid in order to give sufficient strength to each of the containers. The bottoms of the containers are sealed with paraffin wax, the object of using porous containers being to separate or isolate, without insulating, the electrodes of the battery and to insure continuity of the electrolyte. The legs or plates around and in contact with which the red lead is initially deposited, which do not support active material and are merely conductors for the current are tenuous or thin, and fit loosely within the receptacles to leave room for that positive electrode material. The red lead is preliminarily mixed with water and plaster of Paris to form a creamy mass, two parts by volume of red lead and one part by volume of plaster of Paris being found satisfactory proportions to insure setting or solidification. A suitable frame of paraffined wood or metal is used to support and maintain the shape of the containers while being filled. After the material in the containers is set, the legs or plates of the containers are attached to the positive pole pieces and placed in the battery casing, without the electrolyte being present, following which the negative strips, which are also tenuous or thin, and do not support active material are inserted in alternate positions, and a mixture of litharge and plaster, prepared in the same way as the positive materials introduced in the spaces around the containers. The battery is then allowed to stand for 24 hours, after which the negative strips are attached to the negative terminal. The materials and the cups are now covered with a solution of silicate of soda, which is gradually absorbed by the cellulose and the electrode materials, and a current of electricity is passed through the red lead and into and through the litharge, to thereby complete the battery, the period of time required for this purpose being determined by the appearance of the litharge, which, when turned dark gray, indicates that the battery is complete and ready for the introduction of the electrolyte. If the receptacle 1 is opaque, the results

may be determined by reference to previous experiences of the maker with batteries having transparent receptacles. The battery, as thus completed by the electrolytic action of the current, is charged and ready for service. The electrolyte will then be introduced, and will act to eliminate the plaster of Paris or other substances remaining in the pores of the materials.

Although a sulphuric acid electrolyte is preferable, other electrolytes such as a solution of zinc sulphate, may be employed. The battery will, however, act to produce a current of high voltage and amperage, if an electrolyte of the ordinary kind be not employed, the aqueous solution of sodium silicate being itself a satisfactory electrolyte. If the silicate of soda is to be used as an electrolyte, the aqueous solution thereof previously poured in will be retained, but, if another electrolyte is employed, the excess solution will be removed, and said other electrolyte introduced. The electrolyte then appears to be a composite electrolyte, including the silicate of soda retained in the porous constituents of the battery, and possessing new properties, these new properties being indicated by the continued purity or stability of the materials of the electrodes, by the absence of discoloration of the materials of the containers and the electrodes, by the high conductivity of the materials of the electrodes, by the constant ohmic resistance of the electrolyte, by the ability of the battery to prolong the charge-holding period, and by an increase in the voltage of the battery as compared with that of an ordinary battery, which increase approximates one-quarter of a volt. The precise reaction which take place during the formation, the charging and the discharging of the battery are not fully understood, but the phenomena as herein set forth have been definitely ascertained by a prolonged series of experiments. It is, however, believed that the plaster of Paris, as it is expanded by the water of the mixture, produces porosity in the electrode materials; that the disintegration of the plaster of Paris by the acid reduces its volume, thus increasing the capacity of the pores; that the nascent atoms of hydrogen and of oxygen liberated by the electrolysis of the water, respectively reduce the litharge to metallic lead, and change the red lead to peroxide of lead, these products being formed in a porous condition; and that the cellulose of the containers becomes impregnated with silica, which substance is produced by the action of the acid, sodium sulphate which becomes a part of the electrolyte, also being formed. If water decomposition and recombination is the reversible reaction, storing and reproducing energy, the porous electrodes should remain constant as they appear to do, and operate

to occlude the respective constituents of the water. A cell containing the silicate-of-soda electrolyte has a considerably higher voltage than a cell containing a sulphuric-acid electrolyte, but a cell of the latter kind has the greater capacity in ampere-hours. The silicate-of-soda cell gives off only a mixture of ozone and, possibly, hydrogen while being charged, ozone being liberated at the positive electrode, and is, therefore, especially desirable in situations, as in submarines, where it is essential to maintain the purity of the atmosphere, and is desirable also in flash-light batteries wherein the receptacles are composed of metal, the metal which would be acted upon by sulphuric acid, being inert as respects the silicate of soda.

The silicate of soda will function as an electrolyte if it contain any moisture, but an aqueous solution containing 90 parts by volume of water and 10 parts by volume of silicate of soda, is preferable, because a stronger solution hampers the electrolytic action.

The legs or plates which carry the electric current to and from the active materials, may, as already stated, be tenuous or thin, that is to say, only heavy enough to possess mechanical stability, and also to conduct the current without being overheated, contrary to the practice in the ordinary secondary lead battery. In my battery, the active materials are of such low resistance that the cross-sections of the lead legs or plates may be very small, and the active materials actually predominate, a grid not being relied upon for carrying the current. Lead legs are used, however, because the active materials are capable of adhering thereto more certainly than they would cling to another substance.

The negative electrodes of my completed battery are composed of pure lead which, unlike ordinary electrolytically deposited comminuted lead, is in form a single mass composed of fine coherent and integral filaments possessing lustrous surfaces and presenting to the electrolyte large areas of clean metallic surfaces thereby greatly increasing the activity of the battery as compared with batteries in which the lead is in comminuted form. The negative electrode has a slate color, while the positive electrode is brown after forming, and these colors remain unchanged.

A battery constructed in accordance with my invention, will retain its efficiency for an indefinite period of time, or until the terminals of the battery are disconnected by the complete conversion of the metallic lead to spongy lead in the case of the negative electrode, or to peroxide of lead in the case of the positive electrode, there being no disintegration of the masses of active materials such as occurs in ordinary secondary lead

batteries in which the active materials are carried by grids, these active materials being of such low resistance that a conductive path for the current, such as is afforded by the lead grid of an ordinary battery, is not essential. The battery, because of its construction, is about one-third lighter than an ordinary secondary lead battery of the same capacity.

Furthermore, such a battery will not establish the detrimental internal short circuits which, in previous batteries, operate to discharge them, or, if the electrolyte has evaporated; produce destructive sparking between the electrodes, the internal solid elements of the battery being physically connected throughout by the porous material of the containers, thus eliminating or filling the spark gaps which would otherwise be present.

A further advantage results from the fact that my battery has its capacity increased by successive chargings until all of the materials are rendered active, the ratio of the volume of red lead and litharge, and of the active materials produced therefrom, to the volume of lead, being much greater in the present battery than it is in the usual secondary lead battery, and that it remains charged for a much longer period of time than a battery in which heterogeneous portions of the materials establish local short circuits which reduce the active materials to a condition of inactivity.

The battery herein described may be operated indefinitely without incrustation of the electrodes with lead sulphate which is an essential element of an ordinary battery and which, being a poor electrical conductor, seriously interferes with all of the functions of the battery, and has to be scraped off when in excess; and it, furthermore, is an integral unit, the parts of which cannot be surreptitiously replaced by inferior substitutes, although new lead plates or legs may be inserted in holes bored in the material of the positive electrode when the old ones are completely reduced, thus restoring the only part of the battery which is subject to deterioration.

The battery, as hereinbefore set forth, contains a substantially unchangeable electrolyte which does not yield sulphur to combine with portions of the lead to form lead sulphate, and which therefore approximately retains its specific gravity and affords a constant internal resistance during the entire periods of charging and discharging.

The operation of the battery is believed to be dependent upon the dissociation of molecules of water and the recombination of the resulting oxygen and hydrogen atoms which, pending the generation of the electrical current, are occluded in the pores of the respective electrodes, the hydrogen being

- 4
- occluded in the pores of the lead constituting the negative electrode, and the oxygen being occluded in the pores of the peroxide of lead constituting the positive electrode.
- 5 Reasons for believing that the battery operates in this way, are the unchangeability of the electrode materials during the periods of charge and discharge, the constancy of the electrolyte which, as already indicated,
- 10 maintains its specific gravity and its ohmic resistance, and the tidal effect produced in the electrolyte which, during the charging of the battery rises approximately one-half an inch, and which during discharge falls 15 to its normal level or is entirely absorbed by the porous electrodes.

When, in the claims, I refer to "active materials", I mean to include the substances of which the positive and negative electrodes 20 are formed, even though they may not participate in the chemical reactions taking place in the battery; and when, in said claims, I speak of an electrolyte I intend to include any substance which affords a path 25 for the current flowing from one electrode to the other.

The primary battery cell shown in Figure 10 has a retainer 18 of glass or other suitable substance, which may not be inert since 30 the electrolyte 19 is composed of a ten per cent solution of silicate of soda which does not corrode substances that are attacked by acid electrolytes, such as sulphuric acid. The electrodes 20 and 21 are, or may be, respectively composed of carbon and zinc, or 35 other substances which are relatively electro-positive and electro-negative. A primary cell of this type is very efficient. I have found that it has a voltage of 1.5.

40 The ozone or electrolytic cell shown in Figure 9 has a retainer 22 of glass or other desired substance, which may not be inert to acids, positive and negative electrodes 23, 24, which may be carbon rods, and inverted 45 glass tubes or receptacles 25, 26, within which the upper ends of these rods terminate. The electrolyte 27 is a 10% solution of silicate of soda. The current is supplied by a conductor 28 attached to the upper end 50 of the rod 23, and passes out through a conductor 29 attached to the upper end of the rod 24, the electrolyte 27 being included in the current. Bubbles of ozone (probably  $O_3$ ) developed on the surface of the rod 23 55 are caught in the receptacles 25, while bubbles of hydrogen formed on the surface of the rod 24 are caught in the receptacle 26, each receptacle being open at its bottom and closed at its top, valves 30, 31, controlling the escape of the respective gases. The 60 retainer 22 is closed by a suitable cover 32. This electrolytic cell produces large volumes of ozone of abnormal activity, and also large volumes of hydrogen.

65 The volta pile shown in Figure 11 has car-

bon elements 33, and zinc elements 34, and the electrolyte which is a solution of silicate of soda, is held by porous pads 35, of blotting paper.

Having described my invention, what I 70 claim and desire to secure by Letters Patent is;

1. A reversible battery including cellulose container for active material and silicate of 75 soda.

2. A battery including porous cellulose, a solution of silicate of soda, and masses of unformed substances mixed with plaster of Paris.

3. A battery having active material permeated with a metallic salt.

4. A battery having active material permeated with the salt of an alkaline metal.

5. A battery permeated with a sodium salt.

6. A battery permeated with silicate of soda.

7. A lead battery including an electrolyte containing sodium silicate.

8. An occlusive electrode composed of fine 90 coherent and integral filaments.

9. An electrode composed of fine coherent and integral filaments of lead having high occlusive properties.

10. Integral lead for a battery characterized by a high degree of occlusive porosity.

11. An electrode for a lead battery, including active material and a sustaining element for said material composed of cellulose immune to the action of an acid.

12. A lead battery having a single negative electrode surrounding one or more than one positive electrode, and physically connected with said positive electrode by a porous partition constituting a bond for 105 uniting said electrodes.

13. A gridless lead battery in which highly conductive masses of active material constitute substantially the sole conducting path for the current.

14. A battery including positive and negative materials, an electrolyte, and porous cellulose containers for said materials which are inert to an electrolyte, such as sulphuric acid.

15. A reversible lead battery having an electrolyte of constant chemical constitution and constant ohmic resistance.

16. A battery, including electrode materials respectively composed of litharge and red lead, an electrolyte composed of silicate of soda, a cellulose container for electrode material, and a solution of silicate of soda permeating said cellulose.

17. The process of preparing a cellulose 125 container for use in a battery, which consists in passing a current of electricity through silicate of soda in the presence of an undeveloped cellulose container.

18. The process of completing a battery 130

- containing a cellulose container, which consists in saturating said container with a metallic salt, arranging non-active electrode materials in proper relation to said container, and passing a current of electricity through the incomplete battery until it is materially charged and the cellulose is rendered inert to sulphuric acid.
19. The process of treating cellulose for use in a battery, which consists in subjecting said cellulose and silicate of soda to the action of ozone.
20. The process of completing a battery, including a cellulose container for active material, which consists in supplying thereto an aqueous solution of sodium silicate, passing an electric current through the incomplete battery, and continuing said current until the cellulose is rendered chemically inert to the action of an electrolyte.
21. The process of completing a battery including electrodes separated by a porous partition, which consists in supplying thereto an aqueous solution of sodium silicate, passing an electrical current through the incomplete battery, and continuing said current until the materials of the electrodes have become electrically active, or until the battery is substantially charged.
22. The process of producing a battery containing an oxidizable metal and the oxide of a metal, which consists in passing an electrical current through electrode materials and through an associated salt of an alkaline metal in solution.
23. The process of preparing active material for use in a battery, which consists in subjecting said material to the action of an electrical current while in contact with silicate of soda.
24. The process of preparing active material for use in a battery, which consists in the electrolysis of a solution of sodium silicate performed adjacent to said material.
25. The process of producing a battery electrode, which consists in mixing a mass of sub-oxide of lead ( $PhO$ ) in an aqueous solution of a metal silicate, and passing an electric current therethrough.
26. The process of producing an electrode, which consists in mixing with electrode materials a substance, and eliminating said substance to thereby render said electrode materials porous and increase the areas of their active surfaces.
27. The process of producing an electrode, which consists in mixing the electrode materials with plaster of Paris and eliminating said plaster of Paris to thereby render said electrode materials porous and increase the areas of their active surfaces.
28. The process of producing an electrode, which consists in mixing the electrode materials with an alkaline sulphate, and eliminating said sulphate to thereby render said electrode materials porous and increase the areas of their active surfaces.
29. A cell including lead electrodes and the decomposable salt of a metal of the alkali group.
30. A cell including lead electrodes and sodium silicate.
31. A reversible battery comprising active material having constant chemical properties throughout the complete electro-chemical cycle.
32. A gridless battery having a negative electrode substantially composed of porous metallic lead.
33. A gridless battery having a negative mass of porous lead, a positive mass of lead-oxygen composition, and an electrolyte.
34. A gridless battery having a negative mass of porous lead, a positive mass of the peroxide of lead, and an electrolyte.
35. A reversible battery comprising active lead material having constant chemical properties throughout the complete electro-chemical cycle.
36. A reversible battery including a negative electrode of lead, having chemical constancy during both the period of charging and the period of discharging.
37. A reversible battery having a positive electrode of peroxide of lead, having chemical constancy during both the period of charging and period of discharging.
38. A reversible battery having a constant negative electrode of lead, and a positive electrode which in a charged condition of the battery, is an oxide of lead.
39. A reversible battery having in its discharged condition, a porous lead negative electrode.
40. A reversible battery having in its discharged condition, a porous lead negative electrode, and a positive electrode of oxide of lead.
41. A gridless battery cell consisting of two homogeneous masses of lead and of lead composition constituting the active materials, and an electrolyte.
42. A gridless battery cell including homogeneous masses of porous active materials formed of or containing lead, and an electrolyte composed in part of water.
43. An oxy-hydrogen battery including porous electrodes, and water constituting an electrolyte, said electrodes being inert as regards the action of said electrolyte and capable of retaining within their pores oxygen and hydrogen atoms produced by the dissociation of said electrolyte.
44. A reversible lead battery having a composite electrolyte containing sodium sulphate, as a by-product.
45. A chemically inert electrode for a battery characterized by occlusive porosity.
46. The process of forming an electrode

which consists in mixing electrode chemically inert material with a substance to render the completed electrode occlusively porous, and then completing said electrode.

5 47. The process of forming an electrode which consists in mixing electrode chemically inert material with a substance to render the completed electrode occlusively porous, and then completing said electrode

10 by electrolytic action.

48. The process of forming the respective electrodes of a battery, which consists in electrolytically reducing, in the absence of the sulphate radical, litharge to metallic lead, and in electrolytically oxidizing red lead to peroxide of lead.

In witness whereof, I have hereunto set my hand and affixed my seal, this 27th day of June, 1922.

VICTOR C. GOODRIDGE. [L.S.]